

## UNITED STATES PATENT OFFICE

2,492,761

## HIGH-TEMPERATURE ALLOYS

Lee E. Osman, Marblehead, Mass., assignor to  
General Electric Company, a corporation of  
New York

No Drawing. Application November 7, 1947.  
Serial No. 784,757

6 Claims. (Cl. 75—128)

1

This application is a continuation-in-part of my copending application Serial No. 711,471, now abandoned, filed November 21, 1946, as a division of my application Serial No. 595,486, filed May 23, 1945, now Patent 2,442,209, both of which applications are assigned to the same assignee as the present invention.

The present invention is an alloy adapted for use as a wheel material in supercharger turbines and the like.

It is one of the objects of the invention to provide an alloy which develops sufficient strength from heat treatment without cold working.

In my application Serial No. 595,486, Patent 2,442,209, there was disclosed an alloy having a carbon content of 0.25 to 0.35 per cent, about 16 to 18 per cent chromium, about 12 to 14 per cent nickel, about 1.75 to 2.25 per cent molybdenum, about 0.8 to 1.2 per cent tungsten, about 0.4 to 0.6 per cent silicon, about 1.25 to 1.75 per cent manganese, about 0.7 to 1.0 per cent columbium, about 0.45 per cent to 1.20 per cent beryllium, with the balance iron.

The present invention is based in part on the discovery that in order to obtain an alloy of the desired type it is not necessary to hold the proportions of certain of the elements, particularly the nickel, within the limits prescribed in my application Serial No. 595,486, Patent 2,442,209. More specifically I have found that an alloy which will develop sufficient strength from heat treatment without cold working may contain from 0.25 to 0.35 per cent carbon, about 16 to 20 per cent chromium, about 12 to 16 per cent nickel, about 1.75 to 2.25 per cent molybdenum, about 0.8 to 1.2 per cent tungsten, about 0.4 to 0.6 per cent silicon, about 1.0 to 1.75 per cent manganese, about 0.7 to 1.1 per cent columbium, about 0.45 to 1.20 per cent beryllium, with the balance iron.

The alloy may be forged at 2000–2100° F. to 1600–1700° F. In order to develop the optimum properties in the alloy, it is quenched from a temperature of about 1050–1100° C. and thereafter aged for about 15 to 24 hours at 650° C. The alloy as quenched has a Rockwell C hardness of 15 to 20. After aging at 650° C. the Rockwell C hardness is 40 and remains substantially constant at that figure. The alloy does not air harden.

The structure after solution treating and aging consists of a gamma solid solution or a mixture of alpha and gamma solid solutions together with the precipitated compounds and carbides. Precipitated compounds are believed to be complex iron and nickel beryllides. The ratio between the alpha and gamma solid solutions apparently depends on the composition, the nickel-chromium ratio having a decided effect in this respect and also the percentage of beryllium which restricts

the gamma field of the iron-nickel-carbon alloys similar to chromium but to a greater extent.

A solution temperature of 1050° C. provides satisfactory results. If a higher solution temperature is employed, for example, a solution temperature above 1100° C. for example, about 1150° C. there appears to be a tendency toward grain boundary fusion of the beryllium which adversely affects the ductility and also the yield strength and rupture strength of the alloy. The lower solution temperature of 1050° C. avoids this difficulty and also provides material having a higher rupture strength.

Although the maximum hardness in the alloy is obtained with an aging temperature of 500° C., I generally employ an aging temperature of 650° C. since that is usually the maximum operating temperature of supercharger bucket wheels. Above 500° C. the hardness progressively decreases although no considerable decrease is found up to 700° C. However, at 800° C. a substantial softening takes place.

Tensile and rupture properties of a particularly useful alloy (alloy A) comprising a mixture of alpha and gamma solid solutions and consisting of 0.30 per cent carbon, 17 per cent chromium, 13 per cent nickel, 2 per cent molybdenum, 1 per cent tungsten, 0.5 per cent silicon, 1.5 per cent manganese, 0.8 per cent columbium, 1 per cent beryllium with the balance iron, in the form of forged bars which have been heated at 1050° C. for one hour, water quenched and aged at 650° C. for 15 hours and then air cooled, are as follows:

| Bars       | Tested at  | Approximate Proportional Limit | Tensile Strength | Tensile Results |          |
|------------|------------|--------------------------------|------------------|-----------------|----------|
|            |            |                                |                  | Elong.          | Red Area |
| Radial     | Room Temp. | 134,500                        | 176,600          | 7               | 6.93     |
|            | 1000° F.   | —                              | 140,500          | 10              | 14.18    |
|            | 1200° F.   | —                              | 117,000          | 6               | 7.1      |
|            | 1300° F.   | —                              | 104,500          | 5.5             | 7.0      |
|            | 1500° F.   | —                              | 63,000           | 8.5             | 12.7     |
|            | 1500° F.   | 113,650                        | 172,375          | 11.5            | 11.72    |
| Tangential | Room Temp. | —                              | 114,200          | 5               | 13.08    |
|            | 1200° F.   | —                              | 63,185           | 9.5             | 16.01    |
|            | 1500° F.   | —                              | —                | —               | —        |

## Rupture results at 1200° F.

| Hours | Stress, per sq. in. | Elongation, percent |
|-------|---------------------|---------------------|
| 1000  | 70,500              | 14                  |
| 1000  | 46,500              | 8                   |

An increase in the nickel content of the alloy over that of alloy A, that is, an increase in the nickel-chromium ratio, decreases the ratio between the alpha- and gamma-solid solutions or eliminates the alpha-solid solution. For example,

each of the following alloys, after the precipitation heat treatment, are characterized by a microstructure consisting of a matrix of gamma-solid solution with precipitated carbides and beryllides:

| Alloy      | B       | C       | D       | E       |
|------------|---------|---------|---------|---------|
| Carbon     | 0.28    | 0.26    | 0.29    | 0.27    |
| Silicon    | 0.37    | 0.39    | 0.41    | 0.38    |
| Manganese  | 1.20    | 1.18    | 1.13    | 1.57    |
| Chromium   | 17.45   | 18.33   | 18.39   | 19.17   |
| Nickel     | 16.99   | 23.76   | 30.12   | 35.80   |
| Tungsten   | 0.96    | 0.93    | 0.96    | 0.94    |
| Molybdenum | 2.17    | 2.10    | 2.16    | 2.19    |
| Columbium  | 0.91    | 1.02    | 0.96    | 0.89    |
| Beryllium  | 1.04    | 1.02    | 0.86    | 0.89    |
| Iron       | balance | balance | balance | balance |

The forgeabilities of alloys B-E inclusive were good although those with nickel content of more than 30 per cent were slightly more difficult to forge than those with lower nickel contents. The oxidation resistances of all were good up to at least 1300° F.

Tensile properties and rupture results of these alloys in the form of forged bar stock which have been heated at 1050° C. for one hour, water quenched, aged for 15 hours at 650° C. and air quenched are as follows:

#### Tensile results

| Alloy | Tested at— | Yield Strength (.002"")<br>p. s. i. | Tensile Strength,<br>p. s. i. | Elong.,<br>Percent | Red Area,<br>Percent |
|-------|------------|-------------------------------------|-------------------------------|--------------------|----------------------|
| B     | RT         | 73,090                              | 150,820                       | 22                 | 33.1                 |
| B     | 1200° F    |                                     | 108,500                       | 17                 | 33.0                 |
| C     | RT         | 79,220                              | 141,730                       | 17                 | 26.0                 |
| C     | 1200° F    |                                     | 106,600                       | 15.5               | 32.9                 |
| D     | RT         | 71,730                              | 135,170                       | 21.7               | 38.1                 |
| E     | RT         | 83,060                              | 157,250                       | 27.5               | 38.9                 |

#### Rupture results at 1200° F.

| Alloy | Hours | Stress, p. s. i. |
|-------|-------|------------------|
| B     | 100   | 68,000           |
| B     | 1,000 | 40,000           |
| C     | 100   | 62,000           |
| C     | 1,000 | 53,500           |
| D     | 100   | over 70,000      |
| D     | 1,000 | 48,000           |
| E     | 100   | 50,000           |

The alloys B, C and D when heated to 1100° C. for 1 hour, water quenched, aged for 15 hours at 650° C. and air quenched tested as follows:

#### Tensile results

| Alloy | Tested at— | Yield Strength (.002"")<br>p. s. i. | Tensile Strength,<br>p. s. i. | Elong.,<br>Per Cent | Red Area,<br>Per Cent |
|-------|------------|-------------------------------------|-------------------------------|---------------------|-----------------------|
| B     | RT         | 132,260                             | 204,000                       | 7                   | 10.5                  |
| C     | RT         | 109,810                             | 186,250                       | 9                   | 13.5                  |
| D     | RT         | 93,650                              | 181,530                       | 19.3                | 20.1                  |

#### Rupture results at 1200° F.

| Alloy | Hours | Stress, p. s. i. |
|-------|-------|------------------|
| B     | 100   | 66,000           |
| B     | 1,000 | 52,000           |
| C     | 100   | 62,000           |
| C     | 1,000 | 53,500           |
| D     | 100   | 65,000           |
| D     | 1,000 | 58,000           |

In general, the alloys containing less than about 30 per cent, i. e., from about 12 to 30 per cent, nickel are preferred from the standpoint of optimum forgeability and high temperature strength characteristics.

What I claim as new and desire to secure by Letters Patent of the United States, is:

1. A heat treatable iron base alloy containing about 0.25 to 0.35 per cent carbon, about 16 to 20 percent chromium, about 12 to 36 per cent nickel, about 1.75 to 2.25 per cent molybdenum, about 0.8 to 1.2 per cent tungsten, about 0.4 to 0.6 per cent silicon, about 1.00 to 1.75 per cent manganese, about 0.7 to 1.1 per cent columbium, about 0.45 to 1.2 per cent beryllium with the balance substantially all iron.

2. A heat treatable iron base alloy containing about 0.25 to 0.35 per cent carbon, about 16 to 20 per cent chromium, about 12 to 30 per cent nickel, about 1.75 to 2.25 per cent molybdenum, about 0.8 to 1.2 per cent tungsten, about 0.4 to 0.6 per cent silicon, about 1.00 to 1.75 per cent manganese, about 0.7 to 1.1 per cent columbium, about 0.45 to 1.2 per cent beryllium with the balance substantially all iron.

3. A heat treatable iron base alloy containing about 0.25 to 0.35 per cent carbon, about 16 to 18 per cent chromium, about 12 to 14 per cent nickel, about 1.75 to 2.25 per cent molybdenum, about 0.8 to 1.2 per cent tungsten, about 0.4 to 0.6 per cent silicon, about 1.25 to 1.75 per cent manganese, about 0.7 to 1.0 per cent columbium, about 0.45 to 1.2 per cent beryllium with the balance substantially all iron.

4. A heat treatable iron base alloy containing about 0.3 per cent carbon, about 17 per cent chromium, about 13 per cent nickel, about 2 per cent molybdenum, about 1 per cent tungsten, about 0.5 per cent silicon, about 1.5 per cent manganese, about 0.8 per cent columbium, about 1 per cent beryllium with the balance substantially all iron.

5. A heat treatable iron base alloy containing about 0.3 per cent carbon, about 18 per cent chromium, about 24 per cent nickel, about 2 per cent molybdenum, about 1 per cent tungsten, about 0.4 per cent silicon, about 1.2 per cent manganese, about 1.0 per cent columbium, about 1 per cent beryllium with the balance substantially all iron.

6. A heat treatable iron base alloy containing about 0.3 per cent carbon, about 18 per cent chromium, about 30 per cent nickel, about 2 per cent molybdenum, about 1 per cent tungsten, about 0.4 per cent silicon, about 1.1 per cent manganese, about 0.8 per cent columbium, about .9 per cent beryllium with the balance substantially all iron.

LEE E. OSMAN.

#### REFERENCES CITED

The following references are of record in the file of this patent:

#### UNITED STATES PATENTS

Number Name Date  
1,945,653 Masing Feb. 6, 1934  
2,373,490 Mohling Apr. 10, 1945

#### FOREIGN PATENTS

Number Country Date  
392,711 Great Britain May 25, 1933